

## UNITED STATES PATENT OFFICE.

PETER J. McINERNEY, OF DALLAS, TEXAS.

## PROCESS FOR TREATING ASPHALTIC PAVING MATERIALS.

No Drawing.

Application filed July 3, 1925. Serial No. 41,429.

This invention relates to processes for treating asphaltic paving materials and refers more particularly to a process of this character wherein the asphaltic elements are 5 broken up and held in suspension in a semi-solid state or friable condition for extended periods of time.

The principal object of this process is to render the asphaltic material more friable, 10 or easier to handle in shipment, maintaining it in a plastic state until such time as it may be laid on the contract.

Further, by the application of my process, the material may be shipped in open cars, at 15 less expense.

Another advantage is that the application of my process to the material at the source of supply of the material, eliminates all temporary mixing plants in proximity to each 20 individual contract, and enables one mixing plant at the source of supply to supply numerous contracts.

Another feature or advantage is that the filler used in my process, the application of 25 which to the asphaltic material renders the latter more friable, is stored in vats at the source of supply and maintained at a degree of temperature (Fahrenheit) about twenty percent lower than the normal temperature, 30 and is mixed by an even rapid application with the hot asphaltic material in a pug mill or other suitable agency when desired.

In substance, the asphaltic materials, after 35 being mixed in the customary manner, that is, with certain proportions of asphalt, stone and sand, and while still at a very hot temperature, say, from two hundred and fifty to three hundred and seventy five degrees Fahrenheit, has applied thereto simultaneously over the entire surface, a mixture of sand and water or sand and Portland cement and water or sand and stone dust and water or sand and hydrated lime and water at a substantially lowered temperature.

45 This application literally blows the asphalt into a multitude of particles which are held in suspension by the use of the filler and remain in a semi-solid, plastic or friable state until the water evaporates or is vaporized artificially.

Thus it will readily be comprehended that the amount of water used in the filler together with the atmospheric conditions as to 55 temperature will determine the limit of distance and time consumed in transit before the evaporation of the water and the subse-

quent solidification of the material takes place.

When the material arrives at the contract and is laid on the highway, pavement or 60 other surface whereon it is to be used, as it is laid it is raked with hot implements and a surface heater employed when necessary to complete the evaporation of the water before 65 the resultant mass is rolled.

The temperature of the water and other ingredients making up the filler must be of a temperature low enough to balance the temperature of the asphaltic materials, so 70 that the latter may be successfully treated for shipment.

Ordinarily sand and water are employed, but in the case of laying sheet pavements where a certain percentage of the materials are required to pass through a two hundred 75 mesh screen, the Portland cement, stone dust, or hydrated lime mentioned above must be mixed with the cold water and sand before the filler is applied to the asphaltic material, otherwise the Portland cement, stone 80 dust, or hydrated lime, if mixed with the asphaltic material would set before application of the filler.

The stone or sand mixed with the hot asphalt may be either heated or treated as desired. 85

In computing the percentage of asphalt used in the mix, the filler should be computed as part of the original mix.

What I claim is:

1. The hereindescribed process of treating asphaltic paving materials comprised in applying a filler of sand and water at a maintained low temperature to asphaltic paving material at a correspondingly high temperature, with a rapid and equally distributed application. 90

2. The process for rendering asphaltic material friable, by first heating said asphaltic material to a temperature ranging from two hundred and fifty to three hundred and seventy five degrees Fahrenheit, and by then applying thereto in even, rapid, distribution, a filler comprised of sand and water at a temperature low enough to balance the temperature of the asphaltic material and to break up or reduce it to a state of friability. 100

3. In preparing asphaltic paving materials for paving, the process of applying a cold filler comprised of sand and water, with the addition of Portland cement, stone dust, 110

or hydrated lime, thereto, to said asphaltic material, when the latter is in a hot, semi-liquid state, in even, rapid distribution to all exposed surfaces of the asphaltic material.

5 4. A process whereby asphaltic paving material is rendered friable, by applying a filler at a maintained low temperature to the

asphaltic material at a maintained high temperature, in an even rapid distribution to all exposed surfaces of the asphaltic material.

In testimony whereof, I have signed my name to this specification.

PETER J. McINERNEY.